



US006481353B1

(12) **United States Patent**  
Geddes et al.

(10) **Patent No.:** US 6,481,353 B1  
(45) **Date of Patent:** Nov. 19, 2002

(54) **PROCESS FOR PREPARING A CERAMIC DECAL**

(75) Inventors: **Pamela A. Geddes**, Alden, NY (US);  
**Barry J. Briggs**, Kelowna (CA);  
**Daniel J. Harrison**, Pittsford, NY (US)

(73) Assignee: **International Imaging Materials, Inc.**,  
Amherst, NY (US)

(\*) Notice: Subject to any disclaimer, the term of this patent is extended or adjusted under 35 U.S.C. 154(b) by 59 days.

(21) Appl. No.: **09/702,415**

(22) Filed: **Oct. 31, 2000**

(51) **Int. Cl.<sup>7</sup>** ..... **B41F 31/00**

(52) **U.S. Cl.** ..... **101/491; 101/483; 156/277**

(58) **Field of Search** ..... 101/33, 34, 483, 101/487, 488, 491, 492; 156/89.11, 230, 233, 237, 277; 427/145, 147, 148, 149; 428/914

(56) **References Cited**

U.S. PATENT DOCUMENTS

5,665,472 A \* 9/1997 Tanaka et al. ..... 428/195

6,149,747 A 11/2000 Lorenz et al.  
6,206,996 B1 \* 3/2001 Hanoka et al. ..... 136/243  
6,280,552 B1 \* 8/2001 Bottari ..... 156/230  
6,368,696 B1 \* 4/2002 Asahi et al. ..... 428/195

\* cited by examiner

*Primary Examiner*—Ren Yan

(74) *Attorney, Agent, or Firm*—Greenwald & Basch LLP;  
Howard J. Greenwald

(57) **ABSTRACT**

A process for preparing a ceramic decal in which a printed image is applied to a backing sheet, and a covercoating is then applied to the printed substrate. A digitally printed ceramic colorant image is applied to the backing sheet; metal oxide colorant with a refractive index of greater than about 1.6 is used as the colorant. Thereafter, the printed image is covercoated with an overcoat containing frit and binder. The total amount of frit applied in the process divided by the total amount of colorant used is at least 2, and the frit used has a melting temperature of at least 550 degrees Centigrade.

**17 Claims, 13 Drawing Sheets**





**FIG. 1**



**FIG. 2**



**FIG. 3**



**FIG. 4**



**FIG. 5**



**FIG. 6**



**FIG.6A**



FIG. 7



**FIG. 8**

FIG.9





**FIG.11**

## PROCESS FOR PREPARING A CERAMIC DECAL

### FIELD OF THE INVENTION

A dry thermal printing process for printing a color image to a backing sheet which thereafter can be utilized to transfer the image to a ceramic substrate.

### BACKGROUND OF THE INVENTION

Processes for preparing "decals" are well known. Thus, e.g., in U.S. Pat. No. 5,132,165 of Louis A. Blanco, a wet printing technique was described comprising the step of offset printing a first flux layer onto a backing sheet, forming a wet ink formulation free of glass and including a liquid printing vehicle and oxide coloring agent, wet printing the wet ink formulation onto the first flux layer to form a design layer, and depositing a second flux layer onto the design layer.

The process described by this Blanco patent is not readily adaptable to processes involving digital imaging, for the wet inks of this patent are generally too viscous for ink jet printing and not suitably thermoplastic for thermal transfer or electrophotographic printing. Digital printing methodologies offer a more convenient and lower cost method of mass customization of ceramic articles than do conventional analog printing methodologies, but they cannot be effectively utilized by the process of the Blanco patent.

The Blanco patent issued in July of 1992. In September of 1997, U.S. Pat. No. 5,665,472 issued to Konsuke Tanaka. This patent described a dry printing process which overcame some of the disadvantages of the Blanco process. The ink formulations described in the Tanaka patent are dry and are suitable to processes involving digital imaging.

However, although the Tanaka process is an improvement over the Blanco process, it still suffers from several major disadvantages, which are described below.

The Tanaka patent discloses a thermal transfer sheet which allegedly can "... cope with color printing ..." According to Tanaka, "... thermal transfer sheets for multi-color printing also fall within the scope of the invention" (see Column 4, lines 64-67). However, applicants have discovered that, when the Tanaka process is used to prepare digitally printed backing sheets for multi-coloring printing on ceramic substrates, unacceptable results are obtained.

The Tanaka process requires the presence of two "essential components" in a specified glass frit (see lines 4-12 of Column 4). According to claim 1 of U.S. Pat. No. 5,665,472, the specified glass frit consists essentially of 75 to 85 weight percent of  $\text{Bi}_2\text{O}_3$  and 12 to 18 weight percent of  $\text{B}_2\text{O}_3$ , which are taught to be the "essential components" referred to by Tanaka. In the system of this patent, the glass frit and colorant particles are dispersed in the same ink. It is taught that, in order to obtain good dispersibility in this ink formulation, the average particle size of the dispersed particles should be from about 0.1 to about 10 microns (see Column 4 of the patent, at lines 13-17).

In the example presented in the Tanaka patent (at Column 7 thereof), a temperature of 450 degrees Celsius was used to fire images printed directly from thermal transfer sheets made in accordance with the Tanaka process to a label comprised of inorganic fiber cloth coated with some unspecified ceramic material.

When one attempts to use the process of the Tanaka patent to transfer images from a backing sheet to solid ceramic substrates (such as glass, porcelain, ceramic whitewares,

etc.), one must use a temperature in excess of 550 degrees Celsius to effectively transfer an image which is durable. However, when such a transfer temperature is used with the Tanaka process, a poor image comprised with a multiplicity of surface imperfections (such as bubbles, cracks, voids, etc.) is formed. Furthermore, when the Tanaka process is used to attempt to transfer color images, a poor image with low color density and poor durability is formed. The Tanaka process, although it may be useful for printing on flexible ceramic substrates such as glass cloth, is not useful for printing color images on most solid ceramic substrates.

It is an object of this invention to provide a digital process for preparing a decal for transferring images to a ceramic substrate which can effectively and durably transfer an image with improved optical properties.

### SUMMARY OF THE INVENTION

In accordance with this invention, there is provided a digital process for preparing a ceramic decal. In one step of this process, a digitally printed ceramic colorant image is applied to a coated backing sheet utilizing a specified colorant. A flux covercoat is digitally printed to the assembly either before or after the ceramic colorant image has been applied; the covercoat contains both frit and binder, and the frit has a melting temperature of at least 550 degrees Centigrade. The total amount of frit applied to the backing sheet in this process is at least 2 times as great as the total amount of colorant used in the process.

### BRIEF DESCRIPTION DRAWINGS

The invention will be described by reference to this specification and the attached drawings, in which like numerals refer to like elements, and in which:

FIG. 1 is a schematic representation of a ceramic substrate to which a color image has been transferred in accordance with the invention;

Each of FIGS. 2, 3, 4, 5, and 6 is a schematic of a preferred ribbon which may be used to prepare the ceramic substrate of FIG. 1;

FIG. 6A is a schematic representation of another preferred ribbon which may be used to prepare the ceramic substrate of FIG. 1;

Each of FIGS. 7 and 8 is schematic of a preferred decal which may be used to prepare the ceramic substrate of FIG. 1; and

Each of FIGS. 9, 10, 10A, and 11 is a flow diagram illustrating how the ribbon, a first decal, a second decal, and the printed ceramic substrate of the invention, respectively, is made.

### DESCRIPTION OF THE PREFERRED EMBODIMENTS

FIG. 1 is a schematic representation of a printed ceramic substrate 10 made in accordance with one preferred process of this invention. The Figures of this patent application are not necessarily drawn to scale.

Printed ceramic substrate 10 is comprised of a ceramic substrate 12 onto which the color image(s) is fixed.

The ceramic substrate used in the process of this invention preferentially has a melting temperature of at least 550 degrees Centigrade. As used in this specification, the term melting temperature refers to the temperature or range of temperatures at which heterogeneous mixtures, such as a glass batch, glazes, and porcelain enamels, become molten

or softened. See, e.g., page 165 of Loran S. O'Bannon's "Dictionary of Ceramic Science and Engineering" (Plenum Press, New York, 1984). In one embodiment, it is preferred that the substrate have a melting temperature of at least about 580 degrees Centigrade. In another embodiment, such melting temperature is from about 580 to about 1,200 degrees Centigrade.

The ceramic substrate used in the process of this invention preferably is a material which is subjected to a temperature of at least about 540 degrees Celsius during processing and is comprised of one or more metal oxides. Typical of such preferred ceramic substrates are, e.g., glass, ceramic whitewares, enamels, porcelains, etc. Thus, by way of illustration and not limitation, one may use the process of this invention to transfer and fix color images onto ceramic substrates such as dinnerware, outdoor signage, glassware, decorative giftware, architectural tiles, color filter arrays, floor tiles, wall tiles, perfume bottles, wine bottles, beverage containers, and the like.

Referring again to FIG. 1, and in the preferred but optional embodiment depicted therein, it will be seen that a flux underlayer 14 is disposed on top of and bonded to the top surface of the ceramic substrate 12. Flux underlayer 14 is preferably transferred to the ceramic substrate surface at a coating weight (coverage) of at least about 1 gram per square meter. It is preferred to use a coating weight (coverage) for flux layer 14 of at least 7 grams per square meter; and it is more preferred to use a coating weight (coverage) for layer 14 of at least about 14 grams per square meter. As will be apparent to those skilled in the art, the coating weight (coverage) referred to herein (and elsewhere in this specification) is a dry weight, by weight of components which contain less than 1 percent of solvent.

The coating composition used to apply layer 14 onto ceramic substrate 12 must contain frit with a melting temperature of at least about 550 degrees Centigrade. As used in this specification, the term frit refers to a glass which has been melted and quenched in water or air to form small friable particles which then are processed for milling for use as the major constituent of porcelain enamels, fritted glazes, frit chinaware, and the like. See, e.g., page 111 of Loran S. O'Bannon's "Dictionary of Ceramic Science and Engineering," supra.

In one embodiment, the frit used in the process of this invention has a melting temperature of at least about 750 degrees Centigrade. In another embodiment, the frit used in the process of this invention has a melting temperature of at least about 950 degrees Centigrade.

One may use commercially available frits. Thus, by way of illustration and not limitation, one may use a frit sold by the Johnson Matthey Ceramics Inc. (498 Acorn Lane, Downingtown, Pa. 19335) as product number 94C1001 ("Onglaze Unleaded Flux"), 23901 ("Unleaded Glass Enamel Flux"), and the like. One may use a flux sold by the Cerdec Corporation of P.O. Box 519, Washington, Pa. 15301 as product number 9630.

Applicants have discovered that, for optimum results, the melting temperature of the frit used should be either substantially the same as or no more than 50 degrees lower than the melting point of the substrate to which the colored image is to be affixed.

The frit used in the coating composition, before it is melted onto the substrate by the heat treatment process described elsewhere in this specification, preferably has a particle size distribution such that substantially all of the particles are smaller than about 10 microns. In one

embodiment, at least about 80 weight percent of the particles are smaller than 5.0 microns.

One may use many of the frits known to those skilled in the art such as, e.g., those described in U.S. Pat. Nos. 5,562,748, 5,476,894, 5,132,165, 3,956,558, 3,898,362, and the like. Similarly, one may use some of the frits disclosed on pages 70-79 of Richard R. Eppler et al.'s "Glazes and Glass Coatings" (The American Ceramic Society, Westerville, Ohio, 2000).

Referring again to FIG. 1, the flux underlayer 14 preferably is comprised of at least about 25 weight percent of one or more frits, by total dry weight of all components in layer 14. In one embodiment, from about 35 to about 85 weight percent of frit material is used in flux underlayer 14. In another embodiment, from about 65 to about 75 percent of such frit material is used.

It is preferred that the frit material used in layer 14 comprise at least about 5 weight percent, by dry weight, of silica. As used herein, the term silica is included within the meaning of the term metal oxide; and the preferred frits used in the process of this invention comprise at least about 98 weight percent of one or more metal oxides selected from the group consisting of lithium, sodium, potassium, calcium, magnesium, strontium, barium, zinc, boron, aluminum, silicon, zirconium, lead, cadmium, titanium, and the like.

Referring again to FIG. 1, in addition to the frit, layer 14 also is comprised of one or more thermoplastic binder materials in a concentration of from about 0 to about 75 percent, based upon the dry weight of frit and binder in such layer 14. In one embodiment, the binder is present in a concentration of from about 15 to about 35 percent. In another embodiment, the layer 14 is comprised of from about 15 to about 75 weight percent of binder.

One may use any of the thermal transfer binders known to those skilled in the art. Thus, e.g., one may use one or more of the thermal transfer binders disclosed in U.S. Pat. Nos. 6,127,316, 6,124,239, 6,114,088, 6,113,725, 6,083,610, 6,031,556, 6,031,021, 6,013,409, 6,008,157, 5,985,076, and the like. The entire disclosure of each of these United States patents is hereby incorporated by reference into this specification.

By way of further illustration, one may use a binder which preferably has a softening point from about 45 to about 150 degrees Celsius and a multiplicity of polar moieties such as, e.g., carboxyl groups, hydroxyl groups, chloride groups, carboxylic acid groups, urethane groups, amide groups, amine groups, urea, epoxy resins, and the like. Some suitable binders within this class of binders include polyester resins, bisphenol-A polyesters, polyvinyl chloride, copolymers made from terephthalic acid, polymethyl methacrylate, vinylchloride/vinylacetate resins, epoxy resins, nylon resins, urethane-formaldehyde resins, polyurethane, mixtures thereof, and the like.

In one embodiment a mixture of two synthetic resins is used. Thus, e.g., one may use a mixture comprising from about 40 to about 60 weight percent of polymethyl methacrylate and from about 40 to about 60 weight percent of vinylchloride/vinylacetate resin. In this embodiment, these materials collectively comprise the "binder."

In one embodiment, the binder is comprised of polybutylmethacrylate and polymethylmethacrylate, comprising from 10 to 30 percent of polybutylmethacrylate and from 50 to 80 percent of the polymethylmethacrylate. In one embodiment, this binder also is comprised of cellulose acetate propionate, ethylenevinylacetate, vinyl chloride/vinyl acetate, urethanes, etc.

One may obtain these binders from many different commercial sources. Thus, e.g., some of them may be purchased from Dianal America of 9675 Bayport Blvd., Pasadena, Tex. 77507; suitable binders available from this source include "Dianal BR 113" and "Dianal BR 106." Similarly, suitable binders may also be obtained from the Eastman Chemicals Company (Tennessee Eastman Division, Box 511, Kingsport, Tenn.).

Referring again to FIG. 1, in addition to the frit and the binder, the layer 14 may optionally contain from about 0 to about 75 weight of wax and, preferably, 5 to about 20 percent of such wax. In one embodiment, layer 14 is comprised of from about 5 to about 10 weight percent of such wax. Suitable waxes which may be used include camuaba wax, rice wax, beeswax, candelilla wax, montan wax, paraffin wax, microcrystalline waxes, synthetic waxes such as oxidized wax, ester wax, low molecular weight polyethylene wax, Fischer-Tropsch wax, and the like. These and other waxes are well known to those skilled in the art and are described, e.g., in U.S. Pat. No. 5,776,280. One may also use ethoxylated high molecular weight alcohols, long chain high molecular weight linear alcohols, copolymers of alpha olefin and maleic anhydride, polyethylene, polypopylene,

These and other suitable waxes are commercially available from, e.g., the Baker-Hughes Baker Petrolite Company of 12645 West Airport Blvd., Sugarland, Tex.

In one preferred embodiment, camuaba wax is used as the wax. As is known to those skilled in the art, carnauba wax is a hard, high-melting lustrous wax which is composed largely of ceryl palmitate; see, e.g., pages 151-152 of George S. Brady et al.'s "Material's Handbook," Thirteenth Edition (McGraw-Hill Inc., New York, N.Y., 1991). Reference also may be had, e.g., to U.S. Pat. Nos. 6,024,950, 5,891,476, 5,665,462, 5,569,347, 5,536,627, 5,389,129, 4,873,078, 4,536,218, 4,497,851, 4,4610,490, and the like. The entire disclosure of each of these United States patents is hereby incorporated by reference into this specification.

Layer 14 may also be comprised of from about 0 to 16 weight percent of plasticizers adapted to plasticize the resin used. Those skilled in the art are aware of which plasticizers are suitable for softening any particular resin. In one embodiment, there is used from about 1 to about 15 weight percent, by dry weight, of a plasticizing agent. Thus, by way of illustration and not limitation, one may use one or more of the plasticizers disclosed in U.S. Pat. No. 5,776,280 including, e.g., adipic acid esters, phthalic acid esters, chlorinated biphenyls, citrates, epoxides, glycerols, glycol, hydrocarbons, chlorinated hydrocarbons, phosphates, esters of phthalic acid such as, e.g., di-2-ethylhexylphthalate, phthalic acid esters, polyethylene glycols, esters of citric acid, epoxides, adipic acid esters, and the like.

In one embodiment, layer 14 is comprised of from about 6 to about 12 weight percent of the plasticizer which, in one embodiment, is diethyl phthalate. The use of this plasticizing agent is well known and is described, e.g., in U.S. Pat. Nos. 6,121,356, 6,117,572, 6,086,700, 6,060,214, 6,051,171, 6,051,097, 6,045,646, and the like. The entire disclosure of each of these United States patent applications is hereby incorporated by reference into this specification.

Suitable plasticizers may be obtained from, e.g., the Eastman Chemical Company.

Referring again to FIG. 1, and in the preferred embodiment depicted therein, it will be seen that, disposed over flux layer 14, is opacification layer 16. Opacification layer 16 is optional; but, when it is used, it is preferably used at a

coating weight (coverage) of from about 0.5 to about 10 grams per square meter and, more preferably, from about 1 to about 5 grams per square meter.

As is known to those skilled in the art, the opacification layer functions to introduce whiteness or opacity into the substrate by utilizing a substance that disperses in the coating as discrete particles which scatter and reflect some of the incident light. In one embodiment, the opacifying agent is used on a transparent ceramic substrate (such as glass) to improve image contrast properties.

One may use opacifying agents which were known to work with ceramic substrates. Thus, e.g., one may use one or more of the agents disclosed in U.S. Pat. Nos. 6,022,819, 4,977,013 (titanium dioxide), U.S. Pat. No. 4,895,516 (zirconium, tin oxide, and titanium dioxide), U.S. Pat. No. 3,899,346, and the like. The disclosure of each of these United States patents is hereby incorporated by reference into this specification.

One may obtain opacifying agents obtained from, e.g., Johnson Matthey Ceramic Inc., supra, as, e.g., "Superpax Zirconium Opacifier."

The opacification agent used should have a melting temperature at least about 500 degrees Centigrade higher than the melting point of the frit(s) used in layer 14. Generally, the opacification agent(s) have a melting temperature of at least about 1200 degrees Centigrade.

The opacification agent should preferably have a refractive index of greater than 2.0 and, preferably, greater than 2.4.

The opacification agent preferably has a particle size distribution such that substantially all of the particles are smaller than about 10 microns. In one embodiment, at least about 80 weight percent of the particles are smaller than 5.0 microns.

Referring again to FIG. 1, in addition to the opacification agent, opacification layer 16 also is comprised of one or more thermoplastic binder materials in a concentration of from about 0 to about 75 percent, based upon the dry weight of opacification agent and binder in such layer 14. In one embodiment, the binder is present in a concentration of from about 15 to about 35 percent. One may use one or more of the binders described with reference to layer 14. Alternatively, one may use one or more other suitable binders.

In addition to the opacifying agent and the optional binder, one may also utilize the types and amounts of wax that are described with reference to layer 14, and/or different amounts of different waxes. Alternatively, or additionally, one may also use the types and amounts of plasticizer described with reference to layer 14. In general, the only substantive differences between layers 14 and 16 are that the calculations are made with respect to the amount of opacifying agent (in layer 16) and not the amount of frit (as is done in layer 14).

Referring again to FIG. 1, one may optionally use a second flux layer 18 similar in composition and/or concentrations to layer 14. When such a second flux layer is used, it will be disposed over and printed over the opacification layer 16.

Disposed over the flux layer 14 is one or more color images 20. These ceramic colorant image(s) 20 will be disposed over either the ceramic substrate 12 or the flux layer 14, and/or the optional opacification layer 16 when used, and/or the optional second flux layer 18 when used.

It is preferred to apply these color image(s) with a digital thermal transfer printer. Such printers are well known to

those skilled in the art and are described in International Publication No. WO 97/00781, published on Jan. 7, 1997, the entire disclosure of which is hereby incorporated by reference into this specification. As is disclosed in this publication, a thermal transfer printer is a machine which creates an image by melting ink from a film ribbon and transferring it at selective locations onto a receiving material. Such a printer normally comprises a print head including a plurality of heating elements which may be arranged in a line. The heating elements can be operated selectively.

Alternatively, one may use one or more of the thermal transfer printers disclosed in U.S. Pat. Nos. 6,124,944, 6,118,467, 6,116,709, 6,103,389, 6,102,534, 6,084,623, 6,083,872, 6,082,912, 6,078,346, and the like. The disclosure of each of these United States patents is hereby incorporated by reference into this specification.

Digital thermal transfer printers are readily commercially available. Thus, e.g., one may use a printer identified as Gerber Scientific's Edge 2 sold by the Gerber Scientific Corporation of Connecticut. With such a printer, the digital color image(s) may be applied by one or more appropriate ribbon(s) in the manner discussed elsewhere in this specification.

Referring again to FIG. 1, the colorant, or colorants which form image 20 are mixed with one or more of the ingredients listed for the opacification layer, with the exception that the colorant(s) is substituted for the opacifying agent(s). Thus, a mixture of the colorant and/or binder and/or wax and/or plasticizer may be used. As will be apparent to those skilled in the art, no glass frit is used in colorant image 20.

It is this element 20 which is selectively applied by the color printer. One such mixture, comprised of one color, may first be digitally printed, optionally followed by one or more differently colored mixtures. The number of colors one wishes to obtain in element 20 will dictate how many different colors are printed.

Although not willing to be bound to any particular theory, applicants believe that the colorant mixtures applied as element 20 tend to admix to some degree.

The amount of colorant used in the composite 11 should not exceed a certain percentage of the total amount of flux used in such composite, generally being 33.33 percent or less. Put another way, the ratio of the total amount of flux in the composite 11 (which includes layers 14, 18, and 24) to the amount of colorant in element 20, in grams/grams, dry weight, should be at least about 2 and, preferably, should be at least about 3. In one embodiment, such ratio is at least 4.0. In another such embodiment, such ratio of flux/colorant is from about 5 to 6. It is noteworthy that, in the process described in U.S. Pat. No. 5,665,472, such ratio was 0.66 (Example 1 at Column 5), or 0.89 (Example 2 at Columns 5-6), or 1.1 (Example 3 at Column 6). At Column 4 of U.S. Pat. No. 5,665,472 (see lines 44 to 49), the patentee teaches that "The proportion of the weight of the bismuth oxide/borosilicate glass frit to the weight of the colorant is preferably 50 to 200% . . ." Thus, substantially more colorant as a function of the flux concentration is used in the process of such patent than is used in applicants' process.

In another embodiment of the invention, the ratio of frit used in the process to colorant used in the process is at least 1.25.

The unexpected results which obtain when the flux/colorant ratios of this invention are substituted for the flux/colorant ratios of the Tanaka patent, and when the flux and colorant layers are separated, are dramatic. A substantially more durable product is produced by the process of the instant invention.

Furthermore, applicants have discovered that, despite the use of substantial amounts of colorant, the process described in U.S. Pat. No. 5,665,472 does not produce transferred images with good color density. Without wishing to be bound to any particular theory, applicants believe that there is a certain optimal amount of encapsulation and immobilization of colorant and/or dissolution of colorant within the flux which is impeded by high concentrations of colorant.

It is disclosed in U.S. Pat. No. 5,665,472 that "The thermal transfer sheet of the present invention can, of course, cope with color treatment," and this statement is technically true. However, such process does not cope very well and must be modified in accordance with applicants' unexpected discoveries to produce a suitable digitally printed backing sheet with adequate durability and color intensity.

The only colorant disclosed in U.S. Pat. No. 5,665,472 is a fired pigment comprised of ferric oxide, cobalt oxide, and chromium trioxide in what appears to be a spinel structure. It is not disclosed where this pigment is obtained from, or what properties it has.

The colorants which work well in applicants' process preferably each contain at least one metal-oxide. Thus, a blue colorant can contain the oxides of a cobalt, chromium, aluminum, copper, manganese, zinc, etc. Thus, e.g., a yellow colorant can contain the oxides of one or more of lead, antimony, zinc, titanium, vanadium, gold, and the like. Thus, e.g., a red colorant can contain the oxides of one or more of chromium, iron (two valence state), zinc, gold, cadmium, selenium, or copper. Thus, e.g., a black colorant can contain the oxides of the metals of copper, chromium, cobalt, iron (plus two valence), nickel, manganese, and the like. Furthermore, in general, one may use colorants comprised of the oxides of calcium, cadmium, zinc, aluminum, silicon, etc.

Suitable colorants are well known to those skilled in the art. See, e.g., U.S. Pat. Nos. 6,120,637, 6,108,456, 6,106,910, 6,103,389, 6,083,872, 6,077,594, 6,075,927, 6,057,028, 6,040,269, 6,040,267, 6,031,021, 6,004,718, 5,977,263, and the like. The disclosure of each of these United States patents is hereby incorporated by reference into this specification.

By way of further illustration, some of the colorants which can be used in the process of this invention include those described in U.S. Pat. Nos. 6,086,846, 6,077,797 (a mixture of chromium oxide and blue cobalt spinel), U.S. Pat. No. 6,075,223 (oxides of transition elements or compounds of oxides of transition elements), U.S. Pat. No. 6,045,859 (pink coloring element) U.S. Pat. No. 5,988,968 (chromium oxide, ferric oxide), U.S. Pat. No. 5,968,856 (glass coloring oxides such as titania, cesium oxide, ferric oxide, and mixtures thereof), U.S. Pat. No. 5,962,152 (green chromium oxides), U.S. Pat. Nos. 5,912,064, 5,897,885, 5,895,511, 5,820,991 (coloring agents for ceramic paint), U.S. Pat. No. 5,702,520 (a mixture of metal oxides adjusted to achieve a particular color), and the like. The entire disclosure of each of these United States patents is hereby incorporated by reference into this specification.

The ribbons produced by the process of this invention are preferably leach-proof and will not leach toxic metal oxide. This is unlike the prior art ribbons described by Tanaka at Column 1 of U.S. Pat. No. 5,665,472, wherein he states that: "In the case of the thermal transfer sheet containing a glass frit in the binder of the hot-melt ink layer, lead glass has been used as the glass frit, posing a problem that lead becomes a toxic, water-soluble compound." Without wishing to be

bound to any particular theory, applicants believe that this undesirable leaching effect occurs because the prior art combined the flux and colorant into a single layer, thereby not leaving enough room in the formulation for sufficient binder to protect the layer from leaching.

The particle size distribution of the colorant used in layer 20 should preferably be within a relatively narrow range. It is preferred that the colorant have a particle size distribution such that at least about 90 weight percent of its particles are within the range of 0.2 to 20 microns.

The colorant used preferably has a refractive index greater than 1.4 and, more preferably, greater than 1.6; and, furthermore, the colorant should not decompose and/or react with the molten flux when subjected to a temperature in range of from about 550 to about 1200 degrees Celsius.

Referring again to FIG. 1, and the preferred embodiment depicted therein, a flux layer 22 optionally may be disposed over the ceramic colorant image element 20. Thus flux layer, when used, will be comparable to the flux layer 18 but need not necessarily utilize the same reagents and/or concentrations and/or coating weight.

Disposed over the colorant image element 20, and coated either onto such element 20 or the optional flux layer 22, is a flux covercoat 24.

Covercoats are described in the patent art. See, e.g., U.S. Pat. No. 6,123,794 (covercoat used in decal), U.S. Pat. Nos. 6,110,632, 5,912,064, 5,779,784 (Johnson Matthey OPL 164 covercoat composition), U.S. Pat. Nos. 5,779,784, 5,601,675 (screen printed organic covercoat), U.S. Pat. No. 5,328,535 (covercoat for decal), U.S. Pat. No. 5,229,201, and the like. The disclosure of each of these United States patents is hereby incorporated by reference into this specification.

The covercoat 24, in combination with the other flux-containing layers, must provide sufficient flux so that the ratio of flux to colorant is within the specified range. Furthermore, it must apply structural integrity to the ceramic colorant image element 20 so that, as described elsewhere in this specification, when composite 10 is removed from its backing material, it will retain its structural integrity until it is applied to the ceramic substrate.

The covercoat 24 should be substantially water-insoluble so that, after it is contacted with water at 40 degrees Centigrade for 1 minute, less than 0.5 percent will dissolve.

The covercoat 24 should preferably have an elongation before break, as measured by standard A.S.T.M. Test D638-58T, of more than 5 percent.

The covercoat 24 should be applied at a sufficient coating weight to result in a coating weight of at least 2 grams per square meter and, more preferably, at least 5 grams per square meter. The covercoat 24 preferably is comprised of the aforementioned flux and carbonaceous material(s) which, in one preferred embodiment, when subjected to a temperature of 440 degrees Centigrade for at least 5 minutes, will be substantially completely converted to gaseous material. The aforementioned binders, and/or waxes, and/or plasticizers described, e.g., with relation to layers 14, 16, 18, 20, 22, and 24, are suitable carbonaceous materials, and one or more of them may be used in the proportions described with regard to layer 14 to constitute the covercoat.

One may use a covercoat 24 which is similar in composition and structure to the layer 14. In one embodiment, it is preferred that the covercoat 24 be comprised of a binder selected from the group consisting of polyacrylate binders, polymethacrylate binders, polyacetal binders, mixtures thereof, and the like.

Some suitable polyacrylate binders include polybutylacrylate, polyethyl-co-butylacrylate, poly-2-ethylhexylacrylate, and the like.

Some suitable polymethacrylate binders include, e.g., polymethylmethacrylate, polymethylmethacrylate-co-butylacrylate, polybutylmethacrylate, and the like.

Some suitable polyacetal binders include, e.g., polyvinylacetal, polyvinylbutyral, polyvinylfornal, polyvinylacetal-co-butyral, and the like.

10 Covercoat 24 preferably should have a softening point in the range of from about 50 to about 150 degrees Centigrade.

In one embodiment, covercoat 24 is comprised of from 0 to 75 weight percent of frit and from 25 to about 100 weight percent of a material selected from the group consisting of binder, wax, plasticizer and mixtures thereof.

FIG. 2 is a schematic representation of a preferred ribbon which may be used in the process of this invention. Referring to FIG. 2, it will be seen that ribbon 30 is comprised of a flexible substrate 32.

20 Substrate 32 may be any substrate typically used in thermal transfer ribbons such as, e.g., the substrates described in U.S. Pat. No. 5,776,280; the entire disclosure of this patent is hereby incorporated by reference into this specification.

25 In one embodiment, substrate 32 is a flexible material which comprises a smooth, tissue-type paper such as, e.g., 30-40 gauge capacitor tissue. In another embodiment, substrate 32 is a flexible material consisting essentially of synthetic polymeric material, such as poly(ethylene terephthalate) polyester with a thickness of from about 1.5 to about 15 microns which, preferably, is biaxially oriented. Thus, by way of illustration and not limitation, one may use polyester film supplied by the Toray Plastics of America (of 50 Belvere Avenue, North Kingstown, R.I.) as catalog number F53.

30 By way of further illustration, substrate 32 may be any of the substrate films disclosed in U.S. Pat. No. 5,665,472, the entire disclosure of which is hereby incorporated by reference into this specification. Thus, e.g., one may use films of 40 plastic such as polyester, polypropylene, cellophane, polycarbonate, cellulose acetate, polyethylene, polyvinyl chloride, polystyrene, nylon, polyimide, polyvinylidene chloride, polyvinyl alcohol, fluororesin, chlorinated resin, ionomer, paper such as condenser paper and paraffin paper, nonwoven fabric, and laminates of these materials.

45 Affixed to the bottom surface of substrate 32 is backcoating layer 34, which is similar in function to the "backside layer" described at columns 2-3 of U.S. Pat. No. 5,665,472. 50 The function of this backcoating layer 34 is to prevent blocking between a thermal backing sheet and a thermal head and, simultaneously, to improve the slip property of the thermal backing sheet.

55 Backcoating layer 34, and the other layers which form the ribbons of this invention, may be applied by conventional coating means. Thus, by way of illustration and not limitation, one may use one or more of the coating processes described in U.S. Pat. No. 6,071,585 (spray coating, roller coating, gravure, or application with a kiss roll, air knife, or

60 doctor blade, such as a Meyer rod), U.S. Pat. No. 5,981,058 (myer rod coating), U.S. Pat. Nos. 5,997,227, 5,965,244, 5,891,294, 5,716,717, 5,672,428, 5,573,693, 4,304,700, and the like. The entire disclosure of each of these United States patents is hereby incorporated by reference into this specification.

65 Thus, e.g., backcoating layer 34 may be formed by dissolving or dispersing the above binder resin containing

additive (such as a slip agent, surfactant, inorganic particles, organic particles, etc.) in a suitable solvent to prepare a coating liquid. Coating the coating liquid by means of conventional coating devices (such as Gravure coater or a wire bar) may then occur, after which the coating may be dried.

One may form a backcoating layer 34 of a binder resin with additives such as, e.g., a slip agent, a surfactant, inorganic particles, organic particles, etc.

Binder resins usable in the layer 34 include, e.g., cellulosic resins such as ethyl cellulose, hydroxyethylcellulose, hydroxypropylcellulose, methylcellulose, cellulose acetate, cellulose acetate butyrate, and nitrocellulose. Viny resins, such as polyvinylalcohol, polyvinylacetate, polyvinylbutyral, polyvinylacetal, and polyvinylpyrrolidone also may be used. One also may use acrylic resins such as polyacrylamide, polyacrylonitrile-co-styrene, polymethylmethacrylate, and the like. One may also use polyester resins, silicone-modified or fluorine-modified urethane resins, and the like.

In one embodiment, the binder comprises a cross-linked resin. In this case, a resin having several reactive groups, for example, hydroxyl groups, is used in combination with a crosslinking agent, such as a polyisocyanate.

In one embodiment, a backcoating layer 34 is prepared and applied at a coat weight of 0.05 grams per square meter. This backcoating 34 preferably is polydimethylsiloxane-urethane copolymer sold as "SP-2200" by the Advanced Polymer Company of New Jersey.

One may apply backcoating 34 at a coating weight of from about 0.01 to about 2 grams per square meter, with a range of from about 0.02 to about 0.4 grams/square meter being preferred in one embodiment and a range of from about 0.5 to about 1.5 grams per square meter being preferred in another embodiment.

Referring again to FIG. 2, and in the preferred embodiment depicted therein, it will be seen that substrate 32 contains an optional release layer 36 coated onto its top surface of the substrate. The release layer 36, when used, facilitates the release of the ceramic colorant/binder layer 38 from substrate 32 when a thermal ribbon 30 is used to print at high temperatures.

Release layer 36 preferably has a thickness of from about 0.2 to about 2.0 microns and typically is comprised of at least about 50 weight percent of wax. Suitable waxes which may be used include carnauba wax, rice wax, beeswax, candelilla wax, montan wax, paraffin wax, mirocrystalline waxes, synthetic waxes such as oxidized wax, ester wax, low molecular weight polyethylene wax, Fischer-Tropsch wax, and the like. These and other waxes are well known to those skilled in the art and are described, e.g., in U.S. Pat. No. 5,776,280.

In one embodiment, at least about 75 weight percent of layer 36 is comprised of wax. In this embodiment, the wax used is preferably carnauba wax.

Minor amounts of other materials may be present in layer 36. Thus, one may include from about 5 to about 20 weight percent of heat-softening resin which softens at a temperature of from about 60 to about 150 degrees Centigrade. Some suitable heat-softening resins include, e.g., the heat-meltable resins described in columns 2 and of U.S. Pat. No. 5,525,403, the entire disclosure of which is hereby incorporated by reference into this specification. In one embodiment, the heat-meltable resin used is polyethylene-co-vinylacetate with a melt index of from about 40 to about 2500 dg. per minute.

Referring to FIG. 2, and in the preferred embodiment depicted therein, the layer 36 may be omitted and the layer 38 may be directly contiguous with substrate 32.

Ceramic colorant/binder layer 38 is one of the layers used to produce the ceramic colorant image 20. In the process of the invention, a multiplicity of ribbons 30, each one of which preferably contains a ceramic colorant/binder layer 38 with different colorant(s), are digitallyprinted to produce said ceramic colorant image 20. What these ribbons have in common is that they all contain both binder and colorant material of the general type and in the general ratios described for layer 20. In one preferred embodiment, there is substantially no glass frit in layer 20 (i.e., less than about 5 weight percent). The concentrations of colorant and binder, and the types of colorant and binder, need not be the same for each ribbon. What is the same, however, are the types of components in general and their ratios.

FIG. 3 is a schematic representation of a preferred ribbon 40 which is similar to the ribbon 30 depicted in FIG. 2 but differs therefrom in that it utilizes a flux layer 42 instead of the ceramic colorant and binder element 38. The flux layer 42, in general, has similar components, and ratios, as the composition of flux layer 18 (see FIG. 1) and is used to deposit layer 14 and/or layer 18 and/or layer 22 onto the ceramic substrate 12. As will be apparent to those skilled in the art, the precise composition and coating weight of flux layer 42 will depend upon the precise composition and coating weight of the flux layer 14 and/or flux layer 18 and/or flux layer 22 desired.

In the embodiment depicted in FIG. 1, at least 4 separate flux-containing layers are depicted. In general, it is preferred to utilize at least two such layers. In general, the number of layers of flux required will depend upon how much total flux must be used to keep the total flux/colorant ratio in composite 11 at least 2.0.

It is preferred not to dispose all of the flux required in one layer. Furthermore, it is preferred that at least some of the flux be disposed below the ceramic colorant image, and at least some of the flux be disposed above the ceramic colorant image.

In one embodiment, at least 10 weight percent of the total amount of flux used should be disposed on top of ceramic colorant image 20 in one or more flux layers (such as layers 22 and 24). In this embodiment, at least about 50 percent of the total amount of flux should be disposed below ceramic colorant image 20 in one or more of flux layer 18 and/or flux layer 14.

In another embodiment, from about 30 to about 70 weight percent of the entire amount of frit used in the process of this invention is disposed below the ceramic image 20, and from about 70 to about 30 weight percent of the entire amount of frit used in the process of the invention should be disposed above the ceramic image 20. As will be apparent to those skilled in the art, a layer of material which contains frit need not necessarily be contiguous with the ceramic colorant image 20 to be disposed either below or above it. Thus, by way of illustration and not limitation, and referring to FIG. 1, the flux underlayer 14 is not contiguous with the ceramic colorant image 20 but is still disposed below such image.

In one embodiment, from about 40 to about 60 weight percent of the entire amount of frit used in the process of this invention is disposed below the ceramic image 20, and from about 60 to about 40 weight percent of the entire amount of frit used in the process of the invention should be disposed above the ceramic image 20. In yet another embodiment,

from about 75 to about 90 weight percent of the entire amount of frit used in the process of this invention is disposed below the ceramic image 20, and from about 25 to about 10 weight percent of the entire amount of frit used in the process of the invention should be disposed above the ceramic image 20.

If the required amount of flux is not disposed above the ceramic colorant image 20, applicants have discovered that poor color development occurs when cadmium pigments and other pigments are used. Inasmuch as the ceramic substrate 12 (see FIG. 1) is substantially as impervious as a sintered flux layer, applicants do not know precisely why this phenomenon occurs.

For non-cadmium-containing ceramic colorant images, applicants have discovered that acceptable results utilizing a single layer of frit may be obtained so long as the single layer of frit is positioned both above the colorant image 20 and the ceramic substrate 12 and provides a ratio of total frit to ceramic colorant in excess of about 1.25, weight /weight.

FIG. 4 is a schematic of yet another preferred ribbon 50 which is similar in construction to the ribbons depicted in FIGS. 2 and 3 but differs therefrom in containing a different arrangement of layers.

FIG. 5 is a schematic of yet another preferred ribbon 52 which is similar to the ribbons depicted in FIGS. 2, 3, and 4 but differs therefrom in containing a flux covercoat layer 46. As will be apparent to those skilled in the art, the flux covercoat layer 46 may be used to deposit the flux covercoat 24 (see FIG. 1) and, thus, should have a composition similar to the desired covercoat 24.

FIG. 6 is a schematic of yet another preferred ribbon 54 which is similar to the other ribbons depicted but which, additionally, is comprised of opacification layer 48. The opacification layer 48 may be used to print opacification layer 16 (see FIG. 1) and, thus, should contain substantially the same components and ratios as described for layer 16.

FIG. 6A is a schematic representation of another preferred ribbon 60 of the invention which is comprised of backcoating layer 34, polyester support 32, and release layer 36. Disposed on top of release layer 36 are a multiplicity of panels which are disposed at selected locations on top of release layer 36. Using conventional printing techniques, one of such panels (such as panel 42) is first coated onto release layer 36 at the desired location, followed by selective coating of the second panel 48, the third panel 38 etc. Although the panels 42, 48, 38, and 46 have been shown in a particular configuration in FIG. 6A, it will be apparent that other panels and/or other configurations may be used.

To obtain such selective location(s) of the panels, one may a gravure coating press. What is obtained with this process is a ribbon with repeating sequences of various panels, which thus can be utilized in a single head thermal transfer printer to obtain a print image with multiple colors and/or compositions and/or properties.

In this embodiment, it is preferred to use a sequence of 42/48/38/38/38/46 to obtain, with printing operation, and covercoated decal which may be used to produce an image on a ceramic substrate with good print density and good durability.

FIG. 7 is a schematic representation of a ceramic decal 70, which can be produced using one or more of the ribbons depicted in FIGS. 2 through 6A. The various panels 38 shown in FIG. 6A represent one or more ceramic colorant panels used to produce a ceramic colorant image 20.

Referring to FIG. 7, and in the preferred embodiment depicted therein, the ceramic decal 70 is preferably comprised of flexible substrate 72.

Flexible substrate 72 is often referred to as a "backing sheet" in the prior art; see, e.g., U.S. Pat. No. 5,132,165 of Blanco, the entire disclosure of which is hereby incorporated by reference into this specification. Thus, e.g., substrate 72 can include a dry strippable backing or a solvent mount or a water mount slide-off decal. The backing may be of paper or other suitable material such as, e.g., plastic, fabric, and the like. In one embodiment, the backing comprises paper which is coated with a release material, such as dextrine-coated paper. Other possible backing layers include those coated with polyethylene glycol and primary aliphatic oxyethylated alcohols.

By way of further illustration, one may use "Waterslide" paper, which is commercially available paper with a soluble gel coat; such paper may be obtained from Brittians Papers Company of England. This paper is also described in U.S. Pat. Nos. 6,110,632, 5,830,529, 5,779,784, and the like; the entire disclosure of each of these United States patents is hereby incorporated by reference into this specification.

Additionally, one may use heat transfer paper, i.e., commercially available paper with a wax coating possessing a melt point in the range of from about 65 to about 85 degrees Centigrade. Such heat transfer paper is discussed, e.g., in U.S. Pat. Nos. 6,126,669, 6,123,794, 6,025,860, 5,944,931, 5,916,399, 5,824,395, 5,032,449, and the like. The disclosure of each of these United States patents is hereby incorporated by reference into this patent application.

Regardless of what paper is used, it is optionally preferred that a flux layer 74 be either coated to or printed on such paper 72. The thickness of such coating 74 should be at least about 5 microns after such coating has dried, and even more preferably at least about 7 microns. Applicants have discovered that when a coating weight is used which produces a thinner layer 74, poor color development results when cadmium-based ceramic colorants are used. It should be noted that, in the process described in U.S. Pat. No. 5,132,165, a thickness of the "prefused glass flux layer" of only from about 3 to about 4 microns is disclosed.

Referring again to FIG. 7, ceramic colorant images 76 (yellow), and/or 78 (magenta) and/or 80 (cyan) and/or 82 (black) may be digitally printed by sequentially using one or more ribbons 30. Flux layers 42 may optionally be printed by utilizing ribbon 40, which can sequentially print layer 42 in between the various image colors. Alternatively, layer 42 may be printed simultaneously with the image colors by the use of ribbon 50.

The preferred ribbons depicted in FIGS. 2 through 6A afford one a substantial amount of flexibility, when using applicants' process, of preparing decals with many different configurations. As will be apparent, one or more printers equipped with one or more of such ribbons can be controlled by a computer, which can produce a decal with substantially any desired combination of colors, colored patterns, images, and physical properties.

Referring again to FIG. 7, the flux covercoat 46 may be printed by means, e.g., of ribbon 52.

FIG. 8 is a schematic representation of a decal 80 which is similar in many respects to decal 70 (see FIG. 7) but differs therefrom in containing an opacification layer -48 which is similar in function and composition to the opacification layer 48 depicted for ribbon 54 (see FIG. 6); in another embodiment, not shown, the flux underlayer 14 is omitted. It should be noted that, in image 20, a multiplicity of ceramic images may be digitally printed and superimposed on each other to form such image.

FIG. 9 is a flow diagram of one preferred process for preparing a ribbon of this invention. As will be apparent to

## 15

those skilled in the art, the process illustrated may be used to prepare ribbon 30, and/or ribbon 40, and/or ribbon 50, etc.

In step 100, one may prepare a ceramic colorant ink as described in this specification, in accordance with the description, e.g., of layer 38 of FIG. 2. This ink may be used to coat the faceside of polyester support 32 in step 114 (see FIG. 2).

In step 102, one may prepare a flux binder ink as described in this specification; see, e.g., layer 42 of FIG. 3 and its accompanying description. This flux binder ink may be used to either directly coat the faceside of the polyester support 32 in step 112, and/or coat over an optional release layer 36 in step 110.

In step 104, a release layer is prepared as described in this specification; see, e.g., release layer 36 of FIG. 2 and its accompanying description. This release layer 36 may optionally be used in step 110 to coat the face side of the polyester substrate 32.

In step 106, a backcoat ink may be prepared as described in this specification; see, e.g., backcoating layer 34 of FIG. 2 and its accompanying description. This backcoat layer 34 may be used to coat the backside of the polyester substrate in step 108.

In step 114, the faceside of the polyester support 32 may be coated with ceramic colorant ink.

As will be apparent to those skilled in the art, using the combination of steps illustrated in FIG. 9, one may readily prepare one or more of the ribbons illustrated in FIGS. 2 through 5. Furthermore, although not specifically depicted in FIG. 9, one may prepare an opacification layer in accordance with the description of opacification layer 48 (See FIG. 6 and its accompanying description) which may be used to prepare ribbons containing such opacification layer; also see FIG. 6A).

FIG. 10 is a schematic diagram of a preferred process for producing a ceramic decal. In step 120, either heat transfer or Waterslide paper is provided; these papers are described in the specification (see element 72 of FIG. 7 and its accompanying description). A flux and binder layer is either coated or printed on the face of such optional step 122 (see element 74 of FIG. 7 and its accompanying description); and this flux and binder layer, when dried, should be at least about 7 microns thick.

In step 124, one may optionally print an opacification layer onto the flux binder layer described in step 122. This opacification layer corresponds to layer 48 of FIG. 8. It is preferred, when such opacification layer is used in step 122, to print an optional flux/binder layer over the opacification layer in step 126; this optional flux binder layer is described as element 42 of FIG. 8. However, as is illustrated in FIG. 10, the optional flux/binder layer may be omitted, and one may proceed directly from step 124 to step 128. Alternatively, one may omit both the opacification step and the optional flux binder layer step and proceed directly from step 122 to 128.

Whichever pathway one wishes to follow, it is preferred to use a ceramic colorant thermal transfer ribbon 114 in step 128. The preparation of this ribbon was illustrated in FIG. 9.

In step 128, which may optionally be repeated one or more times with different ceramic colorant ribbons 114, an color image is digitally printed using such ribbon 114 and a digital thermal transfer printer. In one embodiment, prints were produced using a Zebra 140XiII thermal transfer printer run at 4 inches per second with energy level settings ranging from 18 to 24.

## 16

The digital image to be printed is composed of one or more primary colors, and such image is evaluated to determine how many printings of one or more ceramic colorants are required to produce the desired image. Thus, in decision step 130, if another printing of the same or a different colored image is required, step 128 is repeated. If no such additional printing is required, one may then proceed to step 132 and/or step 134.

In optional step 132, an optional flux binder layer is printed over the ceramic colorant image produced in step(s) 128. This optional flux binder layer corresponds to element 42 of FIG. 8. Thereafter, either one goes from step 132 to 134, or one goes directly from decision step 130 to step 134. In printing step 134, a flux covercoat corresponding to element 24 of FIG. 8 is printed to complete the decal. As will be apparent to those skilled in the art, one may apply the covercoat over the entire decal (which includes both a printed image and unprinted area[s]). Alternatively, one may apply the covercoat over the entire imaged areas.

Thus, a complete decal is produced in FIG. 10 and now be may be used in FIG. 11 to produce the imaged ceramic article.

FIG. 10A illustrates an alternative process for preparing a decal according to the invention. As will be apparent to those skilled in the art, the process illustrated in FIG. 10A is very similar to the process illustrated in FIG. 10 with several exceptions. In the first place, in the process of FIG. 10A, in step 150 the covercoat is applied or printed to the assembly prior to the time the ceramic colorant image 128 is applied. Thereafter, following the application of ceramic colorant image 128, optional flux binder (step 126), and/or opacifying agent (step 124), and/or flux/binder (step 122) may be applied to form the decal 152.

The process of FIG. 10A may be used, e.g., to print a decal which thereafter may be applied, e.g., to a wine bottle. Thus, e.g., in such an embodiment, the image is preferably removed from the decal with hot silicone pad or a hot silicone roller. Thereafter, the image is retransferred directly onto the ceramic article (wine bottle) and processed as illustrated in FIG. 11.

In the process depicted in FIG. 11, the decal produced in step 134 of FIG. 10 is treated in one of two ways, depending upon whether the substrate comprising the decal is Waterslide or heat transfer paper.

If the substrate comprising the image is Waterslide paper, then the decal is first soaked in hot water (at a temperature of greater than 40 degrees Centigrade. for preferably at least about 30 seconds). In step 138, the image on the Waterslide paper is then separated from the paper in step 140, this image is then placed onto a ceramic substrate and smoothed to remove wrinkles or air bubbles in step 142 and dried; and the image is then "fired." The imaged ceramic substrate is subjected to a temperature of from about 550 to about 1200 degrees Centigrade in step 144.

If, alternatively, the substrate is heat transfer paper, then the decal is heated above the melting point of the wax release layer on the paper in step 146; such temperature is generally from about 50 to about 150 degrees Centigrade. Thereafter, while said wax release layer is still in its molten state, one may remove the ceramic colorant image from the paper in step 148, position the image onto the ceramic article in step 150, and then follow steps 142 and 144 as described hereinabove.

When one wishes to make the ornamental wine bottle referred to hereinabove, the step 148 may be accompanied with the use of the hot silicone pad and/or the hot silicone roller described hereinabove.

## EXAMPLES

The following Examples are presented to illustrate the claimed invention but are not to be deemed limitative thereof. Unless otherwise specified, all parts are by weight and all temperatures are in degrees Centigrade.

## Example 1

In this example, three different flexible substrate elements were prepared in order to print a decal. The first such flexible substrate element was a coated waterslide paper. The second flexible substrate element contained colored oxide material. The third such flexible substrate element contained frit. The latter two flexible substrate elements were used to print a decal onto the coated waterslide paper.

## Preparation of the Colored Oxide Ribbon

A colored oxide flexible substrate element was prepared. A 4.5 micron thick poly (ethylene terephthalate) film was used as a substrate film, and it was backcoated with a polydimethylsiloxane-urethane copolymer sold as "SP-2200" by the Advanced Polymer Company of New Jersey at a coat weight of 0.03 grams per square meter. The copolymer composition was applied with a Myer Rod and dried in an oven, at a temperature of 50 degrees Centigrade for 15 seconds.

A release coating composition was prepared for application to the face coat of the polyester film. To a mixture of 38 grams of reagent grade toluene and 57 grams of reagent grade isopropyl alcohol were charged 0.58 grams of Diacarna 3B (an alpha-olefin sold by the Mitsubishi Kasai Company of Japan), 0.6 grams of EVALEX V577 (an ethylene-vinylacetate resin sold by the DuPont Mitsui and Polymers Company of Japan), and 3.82 grams of "POLYWAX 850" (a polyethylene wax sold by the Baker Hughes Baker Petrolite Company of Sugarland Tex.). This mixture was stirred until the components were fully dissolved. Then it was coated with a Myer Rod at a coating weight of 0.5 grams per square meter and thereafter dried for 15 seconds at 50 degrees Centigrade.

The polyester film, with its backcoating and release coating, then was coated with a colored oxide layer at a coating weight of 3.2 grams per square meter; the colored oxide layer was applied to the release layer. The color coating was prepared by mixing 45.02 grams of hot toluene (at a temperature of 60 degrees Centigrade) with 13.51 grams of a mixture of Dianal BR 106 and Dianal BR 113 binders in weight/weight ratio of 1/3; these binders were purchased from the Dianal America Company of Pasadena, Tex. Thereafter, 25 grams of Chrome Blue pigment (sold by Johnson Matthey Ceramic Inc. of Downington, Pa.) were charged to the mixture. The composition thus produced was mixed with 35 grams of ceramic grinding media and milled on a paint shaker for 15 minutes until substantially all of the particles were smaller than 10 microns. Thereafter, 3.57 grams of Unilin 425 (a wax sold by the Baker Hughes Baker Petrolite Company) were dissolved in sufficient reagent grade methyl ethyl ketone to prepare a 15 percent solution, and this wax solution was then charged to the mixture with stirring, until a homogeneous mixture was obtained. Thereafter the mixture was filtered to separate the filtrate from the grinding media, and the filtrate was then coated onto the release layer of the polyester substrate at a coating weight of 3.2 grams per square meter using a Meyer Rod. The coated substrate thus produced was then dried with a hot air gun.

## Preparation of the Frit Covercoat Ribbon

A polyester film with a backcoat and a release coat was prepared in the manner described above, but a frit covercoat

layer was coated over the release coat instead of the colored oxide layer. This frit covercoat layer was prepared by mixing 42.05 grams of isopropyl alcohol and 42.05 grams of methyl ethyl ketone. This solvent mixture was heated to a temperature of 50 degrees Centigrade, and to this hot solvent mixture were charged 11.36 grams of "BUTVAR 79" (a polyvinylbutyral resin sold by the American Cyanamid Company) and 1.26 grams of cellulose acetate butyrate (CAB 553.04, sold by the Eastman Chemical Company of Kingsport, Tenn.), with mixing. The mixture was then allowed to cool to ambient temperature, and then 3.28 grams of dioctylphthalate were added with mixing. Thereafter 45.36 grams of a frit (sold by the Cerdec Corporation of Washington, Pa. as "product number 9630") were charged to the mixture and mixed. Grinding media was then added to the mixture, and the mixture then was comminuted by shaking it on a paint mixer for 15 minutes until substantially all of its particles were smaller than about 10 microns. Thereafter, the filtrate was separated from the grinding media by filtration, and the filtrate was then coated at a coating weight of 7.0 grams per square meter onto the release coat of the coated polyester film. The coated film was then dried for 15 seconds with an air gun.

## Preparation of a Coated Waterslide Paper

25 A coated waterslide paper was prepared. The waterslide paper was obtained from the Brittain Papers Company of England, and an overcoat composition was prepared to coat onto the gel side of this paper.

To prepare the overcoat composition, 38.5 grams of 30 methyl ethyl ketone and 38.5 grams of isopropyl alcohol were mixed and then heated to a temperature of 60 degrees Centigrade. To this warm solvent mixture were added 10.4 grams of polyvinylbutyral resin (sold as BUTVAR 79 by the American Cyanamid Company) and 1.14 grams of cellulose acetate butyrate (CAB 553.04, Eastman Chemical) with stirring, to prepare a substantially homogeneous solution. Thereafter, 11.44 grams of a frit sold by the Cerdec Corporation of Post Office Box 519, Washington, Pa. as "product number 9630" were added to the mixture, with stirring; this frit is comprised of sodium borosilicate frit. The mixture was then mixed for about 10 minutes, until it was substantially homogeneous.

45 Ceramic grinding media were added to the mixture, and the media and mixture were then shaken on a paint mixer for 16 minutes until the maximum particle size of the particles in the mixture was less than 10 microns. Thereafter, the grinding media were removed from the comminuted mixture by filtration.

The comminuted filtrate was then coated onto the gel face 50 of the waterslide paper at a coating weight (coverage) of 14 grams per square meter. The coated substrate was then allowed to dry under ambient conditions for eight hours.

## Printing of a Decal onto the Waterslide Paper

55 Printing was conducted using a Zebra 140Xill thermal transfer printer. The prints were created at 4 inches per second and at energy levels ranging from 18 to 24. Printing was done directly onto the overcoat of the waterslide paper. A digital color image was first printed using the colored oxide ribbon described in this example, and then a covercoat 60 layer was printed over the digital image by printing with the frit covercoat ribbon of this example.

## Separation of the Printed Decal from the Waterslide Paper

The printed waterslide paper was then immersed in warm (40 degree Centigrade) water for 30 seconds. The decal was then separated from the paper backing, and the decal so separated was then positioned onto a porcelain-coated steel substrate and smoothed to remove bubbles and wrinkles

using a squeegee. The porcelain-coated steel substrate was purchased from High Standard, Inc. of Dublin, N.H.

The decal/substrate assembly was then allowed to dry under ambient conditions for 8 hours. It was then fired by heating it for 10 minutes at a temperature of 454 degrees Centigrade, then increasing the temperature to 690 degrees Centigrade and holding it at this temperature for ten minutes, and then allowing the heated assembly to slowly cool to ambient.

The image on the porcelain-coated steel had excellent color density with good image definition. It also was resistant to abrasion.

#### Example 2

The procedure of Example 1 was substantially repeated with the exception that a red cadmium oxide powder (Cadmium Red pigment, obtained from Johnson Matthey) was used instead of the Chrome Blue pigment of Example 1. The image on the porcelain-coated steel had excellent color density with good image definition, and it was also resistant to abrasion.

#### Example 3

The procedure of Example 1 was substantially repeated with the exception that a black oxide powder (Chrome Black 1795, obtained from Johnson Matthey) was used instead of the Chrome Blue pigment of Example 1. The image on the porcelain-coated steel had excellent color density with good image definition, and it was also resistant to abrasion.

#### Comparative Examples 4-5

In these examples, the procedure of Example 1 was followed with several exceptions. In the first place, the water-slide paper used did not contain the overcoat layer described in Example 1. In the second place, the colorant and the metal-oxide frit were both contained in the same layer (in accordance with the procedure described in U.S. Pat. No. 5,665,472, thus obviating the necessity for using the two separate ribbons disclosed in the experiment of Example 1.

#### Comparative Example 4

The experiment described in this Example was designed to illustrate the process described in U.S. Pat. No. 5,665,472. In the first step of the experiment, a black ink was prepared in substantial accordance with the process of this patent.

The following ingredients were combined in 145 grams of warm (60 degrees Centigrade) toluene: 3.0 grams of ethyl-enevinylacetate ("ELVAX 200W, sold by the duPont deNemours and Company of Wilmington, Del.), 2.5 grams of "SUPERESTER W115" polyester resin (sold by the Arakana Chemical Company of Chicago, Ill.), 10 grams of Diacarna 30B alpha-olefin wax (sold by the Mitsubishi Kasai Company), and 5.0 grams of paraffin Wax HNP10 (sold by the Nippon Seiro Co., Ltd. of Tokyo, Japan). This mixture was melted and stirred until it was substantially homogeneous. Thereafter, to this mixture was charged 22.5 grams of Black Oxide 1795 chrome pigment (sold by Johnson Matthey), and 15 grams of APEC Flux 9630. Ceramic grinding media was then charged to and mixed with this mixture, and this mixture was then milled on a paint shaker for 16 minutes until the maximum particle size was less than 10 microns. To this mixture was then added 46.5 grams of carnauba wax (15 percent in methylethyl ketone). The grinding media was then removed from the mixture by

filtration, A polyester substrate with a release layer was prepared as described in Example 1 of this specification. The black ink filtrate of this Example was then coated onto the release layer at a coating weight of 5 grams per square meter and thereafter dried.

The coated polyester substrate was then used to print a decal on waterslide paper, in substantial accordance with the procedure described in Example 1, with the exception that the water slide paper was not modified by having its gel side coated with a frit-containing layer.

A covercoat was then applied over the printed image. The covercoat was a commercially available covercoat (product number 80-977, sold by Cerdec Corporation), it did not contain any frit, and it was applied to the top of the printed images with a Myer rod. The overcoated decal so prepared was allowed to dry for 8 hours.

The dried decal thus prepared was then removed from the waterslide paper in the manner described in Example 1, affixed to the porcelain coated steel substrate, dried, and fired in same manner as Example 1.

The fired image on the porcelain coated steel substrate had poor color density and very poor abrasion resistance. When it was rubbed with only mild pressure using a finger, it readily degraded.

#### Comparative Example 5

The experiment of this Example was conducted in order to demonstrate the process of European patent document 0308518B1. The procedure of Example 4, was substantially used for this Example, with the exception that frit/colorant weight/weight ratio was substantially in accordance with the process depicted in such European patent document.

In the experiment described in this Example, 21.82 grams of if Apec 9630 Flux and 33.35 grams of Chrome Blue pigment were used. The printing conditions described in Example 1 were used to prepare a decal with the ink onto waterslide paper to which a frit-containing overcoat layer had not been affixed. A frit-containing covercoat was not applied over the printed image, but the covercoat described in the Experiment of Example 4 was used.

The fired image on the porcelain coated steel substrate had poor color density and very poor abrasion resistance. When it was rubbed with only mild pressure using a finger, it readily degraded.

#### Comparative Example 6

The procedure of the experiment of Example 5 was substantially followed, with the exception that 33.35 grams of Cadmium Red pigment were used instead of the 33.35 grams of Chrome Blue pigment. Equally poor results were obtained. The fired image on the porcelain coated steel substrate had poor color density and very poor abrasion resistance. When it was rubbed with only mild pressure using a finger, it readily degraded.

It is to be understood that the aforementioned description is illustrative only and that changes can be made in the apparatus, in the ingredients and their proportions, and in the sequence of combinations and process steps, as well as in other aspects of the invention discussed herein, without departing from the scope of the invention as defined in the following claims.

We claim:

1. A process for preparing a ceramic decal, comprising the steps of sequentially:

(a) applying to a backing sheet a flux covercoat with a first surface comprised of a first mixture comprised of a first

- frit and a second solid carbonaceous binder, wherein said first frit has a melting temperature of at least about 550 degrees Centigrade,
- (b) applying to said first surface of said flux covercoat a digitally printed ceramic colorant image comprised of a colorant composition comprising a second surface, wherein:
1. said colorant composition is comprised of metal oxide pigment with a refractive index greater than about 1.4,
  2. said colorant composition is comprised of a multiplicity of metal oxide pigment particles, at least about about 90 weight percent of which are within the range of about 0.2 to about 20 microns, and
  3. said colorant composition is comprised of a first solid carbonaceous binder,
  4. said second surface of said colorant composition is contiguous with at least a portion of said first surface of said flux covercoat, and
  5. the total amount of frit applied to said backing sheet is at least 2 times as great as the total amount of colorant applied to said backing sheet.
2. The process as recited in claim 1, wherein said digital printing is thermal transfer printing.
3. The process as recited in claim 1, wherein said colorant composition is comprised of less than about 5 weight percent of frit.
4. The process as recited in claim 3, further comprising the step of overprinting said second surface of said ceramic colorant image by a process comprising the steps of applying to said ceramic colorant image a second mixture comprised of a second frit and a third solid carbonaceous binder, wherein said second frit has a melting temperature of at least about 550 degrees Centigrade.
5. The process as recited in claim 4, wherein:
- (a) said second mixture is applied to said ceramic colorant image at a coverage of at least about 10 grams per square meter,
  - (b) said second frit comprises at least about 25 weight percent of said second mixture of said second frit and said third solid carbonaceous binder binder,
  - (c) said flux covercoat is applied to said backing sheet at a coverage of at least 2 grams per square meter,

- (d) said flux covercoat is comprised of at least about 25 weight percent of said first frit, provided that the total amount of frit applied to said backing sheet is at least about 4 times as great as the total amount of colorant applied to said backing sheet.
6. The process as recited in claim 5, wherein each of said first carbonaceous binder, said second carbonaceous binder, and said third carbonaceous binder is comprised of less than about 15 weight percent of liquid.
7. The process as recited in claim 6, wherein at least about 50 weight percent of said total amount of frit applied to said backing sheet is applied as said second frit.
8. The process as recited in claim 7, wherein each of said first frit and said second frit has a particle size distribution such that at least about 90 percent of the particles in such frit are smaller than about 5 microns.
9. The process as recited in claim 8, wherein each of said first frit and said second frit is comprised of at least about 5 weight percent of silica.
10. The process as recited in claim 9, wherein said second mixture is comprised of from about 35 to about 85 weight percent of said second frit.
11. The process as recited in claim 10, wherein said second mixture is comprised of from about 15 to about 35 weight percent of said third solid carbonaceous binder.
12. The process as recited in claim 11, wherein said second mixture is comprised of from about 5 to about 20 weight percent of wax.
13. The process as recited in claim 12, wherein said second mixture is comprised of from about 1 to about 15 weight percent of plasticizing agent.
14. The process as recited in claim 5, further comprising the step of printing an opacifying agent over said ceramic colorant image.
15. The process as recited in claim 14, wherein said opacifying agent has a melting temperature of at least about 1200 degrees Centigrade.
16. The process as recited in claim 15, wherein said opacifying agent has a refractive index greater than 2.0.
17. The process as recited in claim 16, further comprising the step of printing a third mixture comprised of a third frit and a fourth solid carbonaceous binder over said opacifying agent.

\* \* \* \* \*